

# UNITED STATES PATENT OFFICE.

SIMON ULLMO, OF LYONS, FRANCE.

## TANNING COMPOUND.

SPECIFICATION forming part of Letters Patent No. 230,841, dated August 3, 1880.

Application filed November 4, 1879.

*To all whom it may concern:*

Be it known that I, SIMON ULLMO, of Lyons, in the Republic of France, have invented a new and Improved Tanning Compound, of 5 which the following is a specification.

The object of my improved compound is to perform a thorough tanning in a very short time.

My composition consists of the following ingredients, in about the following proportions, which are given in quantity sufficient for one hundred pounds of skins: divi-divi, thirty pounds; garouille, or oak-bark, thirty pounds; alum, thirty pounds; sour barley-flour, fifteen 15 pounds; sulphate of copper, one pound.

The skins, having been subjected to the ordinary operations of "river work," are thrown into a hermetically-closed fulling-mill containing a quantity of water sufficient to cover them 20 entirely, and in which the several ingredients hereinabove mentioned have been dissolved and infused. The skins are turned in the fulling-mill during about twenty-four hours with such speed that the temperature cannot exceed 25 the degree above which it would injure

the skin. After coming out of the fulling mill the skins and the solution are thrown into an ordinary vat, in which they are raised every day for fifteen to twenty days, then laid in bark in an ordinary pit during fifteen to thirty 30 days, according to the thickness or body of the skin. This completes the tanning.

I am aware that divi-divi, oak-bark, alum, barley-flour, and metallic sulphates have been used separately, and that some of the said ingredients have been used together for tanning purposes; but I am not aware that all of the said ingredients have been used together in the proportions stated.

What I claim, and desire to secure by Letters Patent, is—

The herein-described tanning compound, consisting of divi-divi, garouille, or oak-bark, alum, sour barley-flour, and sulphate of copper, in about the proportions herein set forth.

SIMON ULLMO.

Witnesses:

LOUIS BACHELE,  
P. TIBRO.